



US010984939B2

(12) **United States Patent**  
**Endo et al.**

(10) **Patent No.:** **US 10,984,939 B2**  
(45) **Date of Patent:** **Apr. 20, 2021**

(54) **MULTILAYER COIL COMPONENT**

(71) Applicant: **TDK CORPORATION**, Tokyo (JP)

(72) Inventors: **Takashi Endo**, Tokyo (JP); **Kenji Komorita**, Tokyo (JP); **Kunihiko Kawasaki**, Tokyo (JP); **Hidekazu Sato**, Tokyo (JP); **Takashi Suzuki**, Tokyo (JP)

(73) Assignee: **TDK CORPORATION**, Tokyo (JP)

(\*) Notice: Subject to any disclaimer, the term of this patent is extended or adjusted under 35 U.S.C. 154(b) by 0 days.

(21) Appl. No.: **15/419,522**

(22) Filed: **Jan. 30, 2017**

(65) **Prior Publication Data**

US 2018/0218829 A1 Aug. 2, 2018

(51) **Int. Cl.**

**H01F 5/00** (2006.01)  
**H01F 17/00** (2006.01)

(52) **U.S. Cl.**

CPC ..... **H01F 17/0033** (2013.01); **H01F 17/0013** (2013.01); **H01F 2017/0066** (2013.01)

(58) **Field of Classification Search**

CPC . **H01L 2924/19042**; **H01L 2924/30107**; **H01L 23/645**; **H01L 23/5227**; **H01F 17/0013**; **H01F 2017/004**; **H01F 2027/2809**; **H01F 27/2804**; **H01F 2017/0066**

USPC ..... 336/200

See application file for complete search history.

(56)

**References Cited**

**U.S. PATENT DOCUMENTS**

5,479,695 A \* 1/1996 Grader ..... H01F 17/0033  
156/89.28  
6,198,373 B1 \* 3/2001 Ogawa ..... H01F 17/0033  
336/83  
6,839,955 B2 \* 1/2005 Uchikoba ..... H01F 27/027  
228/248.1  
6,855,222 B2 \* 2/2005 Konoue ..... B32B 18/00  
156/89.16  
8,004,381 B2 \* 8/2011 Katayama ..... H01F 17/0013  
252/62.6

(Continued)

**FOREIGN PATENT DOCUMENTS**

CN 101529535 A 9/2009  
JP H04-364710 A 12/1992

(Continued)

*Primary Examiner* — Alexander Talpalatski

*Assistant Examiner* — Joselito Baisa

(74) *Attorney, Agent, or Firm* — Oliff PLC

(57) **ABSTRACT**

A multilayer coil component includes an element body, a coil including a plurality of internal conductors, and a plurality of stress-relaxation spaces. The plurality of internal conductors are separated from each other in a first direction in the element body. Each stress-relaxation space is in contact with a surface of the corresponding internal conductor and powders exist in each stress-relaxation space. The element body includes element body regions located between the internal conductors adjacent to each other in the first direction. Each stress-relaxation space includes a first boundary surface with each internal conductor and a second boundary surface with each element body region. The first boundary surface and the second boundary surface oppose each other in the first direction. A distance between the first boundary surface and the second boundary surface is smaller than a thickness of each element body region in the first direction.

**8 Claims, 16 Drawing Sheets**



| (56)                  | References Cited |         |                 |              |                          |                       |  |
|-----------------------|------------------|---------|-----------------|--------------|--------------------------|-----------------------|--|
| U.S. PATENT DOCUMENTS |                  |         |                 |              |                          |                       |  |
| 8,427,265             | B2 *             | 4/2013  | Hachiya .....   | H01F 17/0013 | 2014/0197917             | A1 *                  |  |
|                       |                  |         |                 | 336/83       |                          | 7/2014 Naito .....    |  |
| 9,373,441             | B2 *             | 6/2016  | Noma .....      | H01F 27/34   | 2015/0099115             | A1 *                  |  |
| 9,711,273             | B2 *             | 7/2017  | Suzuki .....    | H01F 27/255  |                          | 4/2015 Maeda .....    |  |
| 2007/0205956          | A1 *             | 9/2007  | Hashimoto ..... | H01L 23/3114 | 2015/0302980             | A1 *                  |  |
|                       |                  |         |                 | 343/866      |                          | 10/2015 Noma .....    |  |
| 2010/0033286          | A1               | 2/2010  | Katayama et al. |              | 2016/0314891             | A1 *                  |  |
| 2011/0133881          | A1 *             | 6/2011  | Nakajima .....  | H01F 3/14    |                          | 10/2016 Onozaki ..... |  |
|                       |                  |         |                 | 336/200      | 2017/0012015             | A1 *                  |  |
| 2012/0326827          | A1 *             | 12/2012 | Nanjyo .....    | H01F 17/0033 |                          | 1/2017 Tsukao .....   |  |
|                       |                  |         |                 | 336/200      | 2017/0073481             | A1 *                  |  |
| 2013/0002389          | A1               | 1/2013  | Son et al.      |              | 2017/0103842             | A1 *                  |  |
| 2013/0154786          | A1 *             | 6/2013  | Nakajima .....  | H01F 5/003   |                          | 4/2017 Nagai .....    |  |
|                       |                  |         |                 | 336/200      | 2019/0096561             | A1 *                  |  |
| 2013/0221959          | A1 *             | 8/2013  | Oki .....       | G01R 15/207  |                          | 3/2019 Nagai .....    |  |
|                       |                  |         |                 | 324/258      | FOREIGN PATENT DOCUMENTS |                       |  |
| 2013/0222104          | A1 *             | 8/2013  | Kitamura .....  | H01F 41/046  | JP                       | H06-096953 A          |  |
|                       |                  |         |                 | 336/200      | JP                       | H08-064421 A          |  |
| 2014/0145816          | A1 *             | 5/2014  | Sato .....      | H01F 17/0013 | JP                       | 10247603 A *          |  |
|                       |                  |         |                 | 336/208      | JP                       | 2006-253322 A         |  |
|                       |                  |         |                 |              | JP                       | 2013-012741 A         |  |
|                       |                  |         |                 |              | WO                       | 2008/004633 A1        |  |
|                       |                  |         |                 |              |                          | 1/2008                |  |

\* cited by examiner

***Fig. 1***

**Fig.2**

*Fig. 3*

*Fig.4*

*Fig.5*



**Fig. 6**

**Fig. 7**

***Fig. 8***

*Fig.9A**Fig.9B*

Fig. 10



**Fig. 11**



*Fig.12*

*Fig.13*

*Fig.14*



Fig. 15

**Fig. 16**



## 1

## MULTILAYER COIL COMPONENT

## TECHNICAL FIELD

The present invention relates to a multilayer coil component.

## BACKGROUND

Japanese Unexamined Patent Publication No. 2006-253322 discloses a multilayer coil component. The multilayer coil component includes an element body including a magnetic material, a coil including a plurality of internal conductors disposed to be separated from each other in a first direction in the element body, and a stress-relaxation portion formed to surround the entire coil.

The stress-relaxation portion is formed to surround the entire coil. Because the stress-relaxation portion is configured using powder, strength of the element body may be lowered. In a multilayer coil component described in Japanese Unexamined Patent Publication No. H6-96953, the stress-relaxation portion is formed to surround each internal conductor configuring the coil, not the entire coil.

## SUMMARY

In the multilayer coil component described in Japanese Unexamined Patent Publication No. H6-96953, the element body includes an element body region located between the individual internal conductors adjacent to each other in the first direction. A thickness of the element body region in the first direction (hereinafter, simply referred to as the "thickness of the element body region") is smaller than an interval between the individual internal conductors adjacent to each other in the first direction. Therefore, if a thickness of the stress-relaxation portion increases, it is difficult to secure the thickness of the element body region. For example, a cross-section of each internal conductor is decreased without changing a length of a magnetic path, so that the thickness of the element body region can be secured. In which case, direct-current resistance of each internal conductor may increase. Also, the length of the magnetic path is increased without changing the cross-section of each internal conductor, so that the thickness of the element body region can be secured. In which case, the thickness of the element body may increase. That is, miniaturization of the multilayer coil component may not be realized.

When the thickness of the element body region is not sufficiently secured, cracks may occur between the individual internal conductors adjacent to each other in the first direction. When the cracks occur between the individual internal conductors adjacent to each other in the first direction, an interlayer short circuit in which the individual internal conductors short-circuit may occur. For this reason, there is a demand for a multilayer coil component in which the thickness of the element body region is sufficiently secured and internal stress occurring in the element body is relaxed.

An object of one aspect of the present invention is to provide a multilayer coil component in which thicknesses of element body regions are sufficiently secured and internal stress occurring in an element body is relaxed.

A multilayer coil component according to an aspect of the present invention includes an element body including a magnetic material, a coil including a plurality of internal conductors, and a plurality of stress-relaxation spaces. The plurality of internal conductors are separated from each

## 2

other in a first direction in the element body and are electrically connected to each other. Each stress-relaxation space is in contact with a surface of the corresponding internal conductor and powders exist in each stress-relaxation space. The element body includes element body regions located between the internal conductors adjacent to each other in the first direction. Each stress-relaxation space includes a first boundary surface with each internal conductor and a second boundary surface with each element body

region. The first boundary surface and the second boundary surface oppose each other in the first direction. A distance between the first boundary surface and the second boundary surface is smaller than a thickness of each element body region in the first direction.

In the multilayer coil component according to the aspect, the individual stress-relaxation spaces are in contact with the surfaces of the corresponding internal conductors. Therefore, the stress-relaxation spaces exist between the internal conductors adjacent to each other in the first direction and

the element body regions located between the internal conductors. The stress-relaxation spaces relax internal stress occurring in the element body. The internal stress occurs due to a difference of thermal shrinkage rates of the internal conductors and the element body, for example. The distances between the first boundary surfaces and the second boundary surfaces in the stress-relaxation spaces are thicknesses of the stress-relaxation spaces in the first direction (hereinafter, simply referred to as the "thicknesses of the stress-relaxation spaces"). The thicknesses of the stress-relaxation spaces are smaller than thicknesses of the element body regions, which are located between the internal conductors adjacent to each other in the first direction, in the first direction (hereinafter, simply referred to as the "thicknesses of the element body regions"). That is, the thicknesses of the element body regions are larger than the thicknesses of at least the stress-relaxation spaces. Therefore, even when the stress-relaxation spaces exist between the internal conductors adjacent to each other in the first direction and the element body regions located between the internal conductors, the element body regions secure the sufficient thicknesses as compared with the stress-relaxation spaces. As a result, the thicknesses of the element body regions are sufficiently secured, and the internal stress occurring in the element body is relaxed.

In the multilayer coil component according to the aspect, each internal conductor may include a first surface facing one direction of the first direction and a second surface facing the other direction of the first direction. The surface with which each stress-relaxation space is contact may be the first surface. When the stress-relaxation spaces are in contact with the first surfaces, that is, the stress-relaxation spaces are formed on the first surfaces of the internal conductors, the stress-relaxation spaces are formed easily and the thicknesses of the element body regions are secured more easily, as compared with when the stress-relaxation spaces are formed on both the first surfaces and the second surfaces.

In the multilayer coil component according to the aspect, the first surface may have a planar shape. In this case, the stress-relaxation space is in contact with the first surface of the planar shape. Because the first surface on which the stress-relaxation space is formed has the planar shape, the stress-relaxation space is formed easily.

In the multilayer coil component according to the aspect, the first surface may include a first surface portion extending in a direction orthogonal to the first direction and a second surface portion inclined with respect to the first direction and

the first surface portion. Each stress-relaxation space may be in contact with the first surface portion and the second surface portion. In which case, even when the first surface of the internal conductor includes the first surface portion and the second surface portion, the stress-relaxation space is in contact with the first surface portion and the second surface portion. Therefore, the internal stress occurring in the element body is relaxed surely.

In the multilayer coil component according to the aspect, an average particle diameter of the powders may be  $0.1 \mu\text{m}$  or less. In which case, because fluidity of the powders is superior, the powders flexibly follow the behavior according to a difference of thermal shrinkage rates of the element body and the internal conductors. As a result, the internal stress occurring in the element body is relaxed more surely.

In the multilayer coil component according to the aspect, materials of the powders may be  $\text{ZrO}_2$ . In which case,  $\text{ZrO}_2$  is hard to affect the magnetic material (for example, a ferrite material) included in the element body. Because a melting point of  $\text{ZrO}_2$  is higher than a firing temperature of the magnetic material,  $\text{ZrO}_2$  exists surely as the powders.

In the multilayer coil component according to the aspect, each internal conductor may contain metal oxide. When the internal conductor contains the metal oxide, a shrinkage rate at the time of firing conductive paste configuring the internal conductor is small as compared with when the internal conductor does not contain the metal oxide. For this reason, a cross-section of the internal conductor is large. Therefore, even when the cross-section of the internal conductor is large, the stress-relaxation space relaxes the internal stress occurring in the element body.

The present invention will become more fully understood from the detailed description given hereinbelow and the accompanying drawings which are given by way of illustration only, and thus are not to be considered as limiting the present invention.

Further scope of applicability of the present invention will become apparent from the detailed description given hereinafter. However, it should be understood that the detailed description and specific examples, while indicating preferred embodiments of the invention, are given by way of illustration only, since various changes and modifications within the spirit and scope of the invention will become apparent to those skilled in the art from this detailed description.

#### BRIEF DESCRIPTION OF THE DRAWINGS

FIG. 1 is a perspective view illustrating a multilayer coil component according to a first embodiment;

FIG. 2 is an exploded perspective view of the multilayer coil component illustrated in FIG. 1;

FIG. 3 is a plan view illustrating a coil conductor;

FIG. 4 is a plan view illustrating a coil conductor;

FIG. 5 is a plan view illustrating a coil conductor;

FIG. 6 is a cross-sectional view of an element body taken along the line VI to VI of FIG. 1;

FIG. 7 is a diagram illustrating a part of FIG. 6;

FIG. 8 is an exploded perspective view of a multilayer coil component according to a second embodiment;

FIGS. 9A and 9B are plan views illustrating connection conductors;

FIG. 10 is a cross-sectional view of the multilayer coil component according to the second embodiment;

FIG. 11 is an exploded perspective view of a multilayer coil component according to a third embodiment;

FIG. 12 is a plan view illustrating a coil conductor;

FIG. 13 is a plan view illustrating a coil conductor;  
FIG. 14 is a plan view illustrating a coil conductor;  
FIG. 15 is a cross-sectional view of the multilayer coil component according to the third embodiment; and  
FIG. 16 is a diagram illustrating a part of FIG. 15.

#### DETAILED DESCRIPTION

Hereinafter, embodiments of the present invention will be described in detail with reference to the accompanying drawings. In the following description, the same elements or elements having the same functions are denoted with the same reference numerals and overlapped explanation is omitted.

##### First Embodiment

A multilayer coil component 1 according to a first embodiment will be described with reference to FIGS. 1 to 7. FIG. 1 is a perspective view illustrating the multilayer coil component according to the first embodiment. FIG. 2 is an exploded perspective view of the multilayer coil component illustrated in FIG. 1. FIGS. 3 to 5 are plan views illustrating coil conductors. FIG. 6 is a cross-sectional view of an element body taken along the line VI to VI of FIG. 1. FIG. 7 is a diagram illustrating a part of FIG. 6. In FIG. 2, illustration of a plurality of magnetic material layers and external electrodes is omitted. In FIG. 6, illustration of the external electrodes is omitted.

As illustrated in FIG. 1, the multilayer coil component 1 includes an element body 2 and a pair of external electrodes 4 and 5. The external electrodes 4 and 5 are each disposed on both ends of the element body 2.

The element body 2 has a rectangular parallelepiped shape. The element body 2 includes a pair of end surfaces 2a and 2b opposing each other and four side surfaces 2c, 2d, 2e, and 2f, as external surfaces thereof. The four side surfaces 2c, 2d, 2e, and 2f extend in a direction in which the end surface 2a and the end surface 2b oppose each other, to connect the pair of end surfaces 2a and 2b. The side surface 2d is a surface opposing other electronic apparatus (for example, a circuit board or an electronic component) not illustrated in the drawings, when the multilayer coil component 1 is mounted on other electronic apparatus.

The direction in which the end surface 2a and the end surface 2b oppose each other, a direction in which the side surface 2c and the side surface 2d oppose each other, and a direction in which the side surface 2e and the side surface 2f oppose each other are approximately orthogonal to each other. The rectangular parallelepiped shape includes a shape of a rectangular parallelepiped in which a corner portion and a ridge portion are chamfered and a shape of a rectangular parallelepiped in which a corner portion and a ridge portion are rounded.

The element body 2 is configured by laminating a plurality of magnetic material layers 11 (refer to FIGS. 3 to 6). The plurality of magnetic material layers 11 are laminated in the direction in which the side surface 2c and the side surface 2d oppose each other. That is, a direction in which the plurality of magnetic material layers 11 are laminated is matched with the direction in which the side surface 2c and the side surface 2d oppose each other. Hereinafter, the direction in which the plurality of magnetic material layers 11 are laminated (that is, the direction in which the side surface 2c and the side surface 2d oppose each other) is also referred to as the "lamination direction". Each of the plurality of magnetic material layers 11 has an approximately

rectangular shape. In the first embodiment, a direction toward the side surface  $2d$  from the side surface  $2c$  is one direction D1 of the lamination direction and a direction toward the side surface  $2c$  from the side surface  $2d$  is the other direction D2 of the lamination direction.

Each magnetic material layer 11 includes a sintered body of a green sheet including a magnetic material (a Ni—Cu—Zn based ferrite material, a Ni—Cu—Zn—Mg based ferrite material, or a Ni—Cu based ferrite material), for example. In the actual element body 2, the individual magnetic material layers 11 are integrated to a degree to which inter-layer boundaries cannot be visualized (refer to FIG. 6). A Fe alloy may be included in the green sheet configuring the magnetic material layer 11.

The external electrode 4 is disposed on the end surface  $2a$  of the element body 2 and the external electrode 5 is disposed on the end surface  $2b$  of the element body 2. That is, the external electrode 4 and the external electrode 5 are separated from each other in the direction in which the end surface  $2a$  and the end surface  $2b$  oppose each other. Each of the external electrodes 4 and 5 has an approximately rectangular shape in planar view and corners of the external electrodes 4 and 5 are rounded. The external electrodes 4 and 5 include a conductive material (for example, Ag or Pd). The external electrodes 4 and 5 include sintered bodies of conductive paste including conductive metal powder (for example, Ag powder or Pd powder) and glass frit. Electroplating is performed on the external electrodes 4 and 5 and plating layers are formed on surfaces of the external electrodes 4 and 5. When the electroplating is performed, for example, Ni or Sn is used.

The external electrode 4 includes five electrode portions. That is, the external electrode 4 includes an electrode portion  $4a$  located on the end surface  $2a$ , an electrode portion  $4b$  located on the side surface  $2d$ , an electrode portion  $4c$  located on the side surface  $2c$ , an electrode portion  $4d$  located on the side surface  $2e$ , and an electrode portion  $4e$  located on the side surface  $2f$ . The electrode portion  $4a$  covers an entire surface of the end surface  $2a$ . The electrode portion  $4b$  covers a part of the side surface  $2d$ . The electrode portion  $4c$  covers a part of the side surface  $2c$ . The electrode portion  $4d$  covers a part of the side surface  $2e$ . The electrode portion  $4e$  covers a part of the side surface  $2f$ . The five electrode portions  $4a$ ,  $4b$ ,  $4c$ ,  $4d$ , and  $4e$  are integrally formed.

The external electrode 5 includes five electrode portions. That is, the external electrode 5 includes an electrode portion  $5a$  located on the end surface  $2b$ , an electrode portion  $5b$  located on the side surface  $2d$ , an electrode portion  $5c$  located on the side surface  $2c$ , an electrode portion  $5d$  located on the side surface  $2e$ , and an electrode portion  $5e$  located on the side surface  $2f$ . The electrode portion  $5a$  covers an entire surface of the end surface  $2b$ . The electrode portion  $5b$  covers a part of the side surface  $2d$ . The electrode portion  $5c$  covers a part of the side surface  $2c$ . The electrode portion  $5d$  covers a part of the side surface  $2e$ . The electrode portion  $5e$  covers a part of the side surface  $2f$ . The five electrode portions  $5a$ ,  $5b$ ,  $5c$ ,  $5d$ , and  $5e$  are integrally formed.

As illustrated in FIGS. 2 to 6, the multilayer coil component 1 includes a plurality of coil conductors 21, 22, and 23 (a plurality of internal conductors), a plurality of connection conductors 24 and 25, and a plurality of stress-relaxation spaces 31, 32, and 33, which are provided in the element body 2. In FIG. 2, the individual stress-relaxation spaces 31 to 33 are shown by dashed-dotted lines.

The coil conductors 21 to 23 and the connection conductors 24 and 25 are separated from each other in the lamination direction (first direction). The thicknesses of the coil conductors 21 to 23 and the connection conductors 24 and 25 in the lamination direction are approximately the same (refer to FIG. 6). Ends of the individual coil conductors 21 to 23 are connected by corresponding through-hole conductors 12b and 12c. An end T1 of the coil conductor 21 and an end T2 of the coil conductor 22 are connected by the through-hole conductor 12b. An end T3 of the coil conductor 22 and an end T4 of the coil conductor 23 are connected by the through-hole conductor 12c. The individual ends T1 to T4 of the coil conductors 21 to 23 are connected via the corresponding through-hole conductors 12b and 12c, so that a coil 20 is configured in the element body 2. That is, the multilayer coil component 1 includes the coil 20 in the element body 2. The coil 20 includes the plurality of coil conductors 21 to 23 that are separated from each other in the lamination direction and are electrically connected to each other. The coil 20 has an axial center along the lamination direction.

The coil conductor 21 is disposed at a position closest to the side surface  $2c$  of the element body 2 in the lamination direction among the plurality of coil conductors 21 to 23. An end E1 of the coil conductor 21 configures one end E1 of the coil 20. The coil conductor 23 is disposed at a position closest to the side surface  $2d$  of the element body 2 in the lamination direction among the plurality of coil conductors 21 to 23. An end E2 of the coil conductor 23 configures the other end E2 of the coil 20. A cross-sectional shape of each of the coil conductors 21 to 23 is approximately a trapezoidal shape (refer to FIG. 6). The cross-sectional shape of each of the coil conductors 21 to 23 is described in detail later with reference to FIG. 7.

The connection conductor 24 is disposed closer to the side surface  $2c$  of the element body 2 than the coil conductor 21 in the lamination direction. The connection conductor 24 and the coil conductor 21 are adjacent to each other in the lamination direction. An end T5 of the connection conductor 24 is connected to the end E1 of the coil conductor 21 by a through-hole conductor 12a. That is, the connection conductor 24 and the end E1 of the coil 20 are connected by the through-hole conductor 12a.

An end 24a of the connection conductor 24 is exposed to the end surface  $2b$  of the element body 2. The end 24a is connected to the electrode portion  $5a$  covering the end surface  $2b$ . That is, the connection conductor 24 and the external electrode 5 are connected. Therefore, the end E1 of the coil 20 and the external electrode 5 are electrically connected via the connection conductor 24 and the through-hole conductor 12a.

The connection conductor 25 is disposed closer to the side surface  $2d$  of the element body 2 than the coil conductor 23 in the lamination direction. The connection conductor 25 and the coil conductor 23 are adjacent to each other in the lamination direction. An end T6 of the connection conductor 25 is connected to the end E2 of the coil conductor 23 by the through-hole conductor 12d. That is, the connection conductor 25 and the end E2 of the coil 20 are connected by the through-hole conductor 12d.

An end 25a of the connection conductor 25 is exposed to the end surface  $2a$  of the element body 2. The end 25a is connected to the electrode portion  $4a$  of the external electrode 4 covering the end surface  $2a$ . That is, the connection conductor 25 and the external electrode 4 are connected. Therefore, the end E2 of the coil 20 and the external electrode 4 are connected.

electrode 4 are electrically connected via the connection conductor 25 and the through-hole conductor 12d.

The coil conductors 21 to 23, the connection conductors 24 and 25, and the through-hole conductors 12a to 12d include a conductive material (for example, Ag or Pd). The coil conductors 21 to 23, the connection conductors 24 and 25, and the through-hole conductors 12a to 12d include sintered bodies of conductive paste including conductive metal powder (for example, Ag powder or Pd powder). The coil conductors 21 to 23, the connection conductors 24 and 24, and the through-hole conductors 12a and 12d may contain metal oxide (TiO<sub>2</sub>, Al<sub>2</sub>O<sub>3</sub>, or ZrO<sub>2</sub>), for example. In which case, the coil conductors 21 to 23, the connection conductors 24 and 24, and the through-hole conductors 12a and 12d include sintered bodies of conductive paste including the metal oxide. In the conductive paste including the metal oxide, a shrinkage rate at the time of firing is small as compared with conductive paste not including the metal oxide.

The individual stress-relaxation spaces 31, 32, and 33 are in contact with the corresponding coil conductors 21 to 23. The stress-relaxation spaces 31 to 33 are spaces where powders 31c, 32c, and 33c exist, respectively. The individual stress-relaxation spaces 31 to 33 exist between the corresponding coil conductors 21 to 23 and element body regions in the element body 2 and relax internal stress occurring in the element body 2. A material of the powders 31c, 32c, and 33c is ZrO<sub>2</sub>, for example. A melting point of ZrO<sub>2</sub> is about 2700° C. or more, for example, and is higher than a firing temperature of a ferrite material. An average particle diameter of the powders 31c, 32c, and 33c is 0.1 μm or less, for example.

The stress-relaxation space 31 is located between the coil conductor 21 and the coil conductor 22 in the lamination direction. As illustrated in FIG. 3, the stress-relaxation space 31 is formed on a surface 21d of the coil conductor 21 (refer to FIG. 7). The surface 21d is a lower surface of the coil conductor 21 in the lamination direction. That is, the surface 21d is a surface close to the side surface 2d in the lamination direction. The stress-relaxation space 31 is formed along a portion other than the end T1 of the coil conductor 21. That is, the stress-relaxation space 31 does not cover the end T1 of the coil conductor 21. The end T1 is a connection portion with the through-hole conductor 12b. The stress-relaxation space 31 is formed not to protrude from the coil conductor 21, when viewed from the lamination direction.

The stress-relaxation space 32 is located between the coil conductor 22 and the coil conductor 23 in the lamination direction. As illustrated in FIG. 4, the stress-relaxation space 32 is formed on a surface 22d of the coil conductor 22 (refer to FIG. 7). The surface 22d is a lower surface of the coil conductor 22 in the lamination direction. That is, the surface 22d is a surface close to the side surface 2d in the lamination direction. The stress-relaxation space 32 is formed along a portion other than the end T3 of the coil conductor 22. That is, the stress-relaxation space 32 does not cover the end T3 of the coil conductor 22. The end T3 is a connection portion with the through-hole conductor 12c. The stress-relaxation space 32 is formed not to protrude from the coil conductor 22, when viewed from the lamination direction.

The stress-relaxation space 33 is located between the coil conductor 23 and the connection conductor 25 in the lamination direction. As illustrated in FIG. 5, the stress-relaxation space 33 is formed on a surface 23d of the coil conductor 23 (refer to FIG. 7). The surface 23d is a lower surface of the coil conductor 23 in the lamination direction. That is, the surface 23d is a surface close to the side surface

2d in the lamination direction. The stress-relaxation space 33 is formed along a portion other than the end E2 of the coil conductor 23. That is, the stress-relaxation space 33 does not cover the end E2 of the coil conductor 23. The end E2 is a connection portion with the through-hole conductor 12d. The stress-relaxation space 33 is formed not to protrude from the coil conductor 23, when viewed from the lamination direction.

As illustrated in FIG. 6, the element body 2 includes element body regions 11a to 11d between the coil conductors 21 to 23 and the connection conductors 24 and 25 adjacent to each other in the lamination direction. The element body region 11a is located between the coil conductor 21 and the coil conductor 22. The element body region 11a is interposed by the stress-relaxation space 31 and the coil conductor 22. The element body region 11b is located between the coil conductor 22 and the coil conductor 23. The element body region 11b is interposed by the stress-relaxation space 32 and the coil conductor 23. The element body region 11c is located between the coil conductor 23 and the connection conductor 25. The element body region 11c is interposed by the stress-relaxation space 33 and the connection conductor 25. The element body region 11d is located between the coil conductor 21 and the connection conductor 24. The element body region 11d is interposed by the coil conductor 21 and the connection conductor 24.

Referring to FIG. 7, cross-sectional configurations of each of the coil conductors 21 to 23 and each of the stress-relaxation spaces 31 to 33 will be described. In FIG. 7, regions including parts (portions close to the end surface 2a of the element body 2) of the coil conductors 21 to 23 in FIG. 6 are expanded. Because configurations of regions including portions of the coil conductors 21 to 23 close to the end surface 2b of the element body 2 in FIG. 6 are the same as the configurations illustrated in FIG. 7, illustration is omitted.

As illustrated in FIG. 7, the coil conductor 21 includes surfaces 21d and 21e. The surface 21d faces the side of the side surface 2d of the element body 2 and the surface 21e faces the side of the side surface 2c of the element body 2. That is, in the first embodiment, the surface 21d is a first surface facing one direction D1 of the lamination direction and the surface 21e is a second surface facing the other direction D2 of the lamination direction. The surface 21d has a planar shape and is approximately orthogonal to the lamination direction. The surface 21e includes a planar portion 21a (first surface portion) and two inclined portions 21b and 21c (second surface portions).

The planar portion 21a has a planar shape and is approximately parallel to the surface 21d. That is, the planar portion 21a extends in a direction orthogonal to the lamination direction. An area of the planar portion 21a is smaller than an area of the surface 21d. Each of the inclined portions 21b and 21c has an inclined shape and is inclined with respect to the lamination direction and the surface 21d. The inclined portion 21b and the inclined portion 21c oppose each other. The inclined portion 21b and the inclined portion 21c are formed to connect the surface 21d and the planar portion 21a. The inclined portion 21b includes a first edge in one direction D1 of the lamination direction and a second edge in the other direction D2 of the lamination direction. The inclined portion 21b is inclined in such a manner that the first edge is closer to the end surface 2a than the second edge. The inclined portion 21c includes a first edge in one direction D1 of the lamination direction and a second edge in the other direction D2 of the lamination direction. The

inclined portion **21c** is inclined in such a manner that the first edge is closer to the end surface **2b** than the second edge. That is, the inclined portion **21b** and the inclined portion **21c** are inclined to come close to each other in the other direction **D2** of the lamination direction.

The coil conductor **22** includes surfaces **22d** and **22e**. The surface **22d** faces the side of the side surface **2d** of the element body **2** and the surface **22e** faces the side of the side surface **2c** of the element body **2**. That is, in the first embodiment, the surface **22d** is a first surface facing one direction **D1** of the lamination direction and the surface **22e** is a second surface facing the other direction **D2** of the lamination direction. The surface **22d** has a planar shape and is approximately orthogonal to the lamination direction. The surface **22e** includes a planar portion **22a** (first surface portion) and two inclined portions **22b** and **22c** (second surface portions).

The planar portion **22a** has a planar shape and is approximately parallel to the surface **22d**. That is, the planar portion **22a** extends in a direction orthogonal to the lamination direction. An area of the planar portion **22a** is smaller than an area of the surface **22d**. Each of the inclined portions **22b** and **22c** has an inclined shape and is inclined with respect to the lamination direction and the surface **22d**. The inclined portion **22b** and the inclined portion **22c** oppose each other. The inclined portion **22b** and the inclined portion **22c** are formed to connect the surface **22d** and the planar portion **22a**. The inclined portion **22b** includes a first edge in one direction **D1** of the lamination direction and a second edge in the other direction **D2** of the lamination direction. The inclined portion **22b** is inclined in such a manner that the first edge is closer to the end surface **2a** than the second edge. The inclined portion **22c** includes a first edge in one direction **D1** of the lamination direction and a second edge in the other direction **D2** of the lamination direction. The inclined portion **22c** is inclined in such a manner that the first edge is closer to the end surface **2b** than the second edge. That is, the inclined portion **22b** and the inclined portion **22c** are inclined to come close to each other in the other direction **D2** of the lamination direction.

The coil conductor **23** includes surfaces **23d** and **23e**. The surface **23d** faces the side of the side surface **2d** of the element body **2** and the surface **23e** faces the side of the side surface **2c** of the element body **2**. That is, in the first embodiment, the surface **23d** is a first surface facing one direction **D1** of the lamination direction and the surface **23e** is a second surface facing the other direction **D2** of the lamination direction. The surface **23d** has a planar shape and is approximately orthogonal to the lamination direction. The surface **23e** includes a planar portion **23a** (first surface portion) and two inclined portions **23b** and **23c** (second surface portions).

The planar portion **23a** has a planar shape and is approximately parallel to the surface **23d**. That is, the planar portion **23a** extends in a direction orthogonal to the lamination direction. An area of the planar portion **23a** is smaller than an area of the surface **23d**. Each of the inclined portions **23b** and **23c** has an inclined shape and is inclined with respect to the lamination direction and the surface **23d**. The inclined portion **23b** and the inclined portion **23c** oppose each other. The inclined portion **23b** and the inclined portion **23c** are formed to connect the surface **23d** and the planar portion **23a**. The inclined portion **23b** includes a first edge in one direction **D1** of the lamination direction and a second edge in the other direction **D2** of the lamination direction. The inclined portion **23b** is inclined in such a manner that the first edge is closer to the end surface **2a** than the second

edge. The inclined portion **23c** includes a first edge in one direction **D1** of the lamination direction and a second edge in the other direction **D2** of the lamination direction. The inclined portion **23c** is inclined in such a manner that the first edge is closer to the end surface **2b** than the second edge. That is, the inclined portion **23b** and the inclined portion **23c** are inclined to come close to each other in the other direction **D2** of the lamination direction.

The stress-relaxation space **31** includes a first boundary surface **31a** with the coil conductor **21** and a second boundary surface **31b** with the element body region **11a**. The first boundary surface **31a** is in contact with the surface **21d** of the coil conductor **21**. The second boundary surface **31b** is in contact with the element body region **11a**. The first boundary surface **31a** and the second boundary surface **31b** oppose each other in the lamination direction.

The stress-relaxation space **32** includes a first boundary surface **32a** with the coil conductor **22** and a second boundary surface **32b** with the element body region **11b**. The first boundary surface **32a** is in contact with the surface **22d** of the coil conductor **22**. The second boundary surface **32b** is in contact with the element body region **11b**. The first boundary surface **32a** and the second boundary surface **32b** oppose each other in the lamination direction.

The stress-relaxation space **33** includes a first boundary surface **33a** with the coil conductor **23** and a second boundary surface **33b** with the element body region **11c**. The first boundary surface **33a** is in contact with the surface **23d** of the coil conductor **23**. The second boundary surface **33b** is in contact with the element body region **11c**. The first boundary surface **33a** and the second boundary surface **33b** oppose each other in the lamination direction.

The thicknesses (hereinafter, simply referred to as the "thicknesses **La**") of the stress-relaxation spaces **31** to **33** in the lamination direction are defined as distances between the first boundary surfaces **31a** to **33a** and the second boundary surfaces **31b** to **33b** opposing each other. In the first embodiment, the thickness **La** of the stress-relaxation space **31** is a distance between the first boundary surface **31a** and the second boundary surface **31b**. The thickness **La** of the stress-relaxation space **32** is a distance between the first boundary surface **32a** and the second boundary surface **32b**. The thickness **La** of the stress-relaxation space **33** is a distance between the first boundary surface **33a** and the second boundary surface **33b**. The thicknesses **La** of the individual stress-relaxation spaces **31** to **33** are equivalent. The same does not necessarily mean only that values are exactly equal. Even when minute differences in a predetermined range or manufacturing errors are included in the values, it may be assumed that the values are the same.

The thicknesses (hereinafter, simply referred to as the "thicknesses **Lb**") of the element body regions **11a** and **11b** in the lamination direction are defined as shortest distances of the element body regions **11a** and **11b** in the lamination direction. In the first embodiment, the thickness **Lb** of the element body region **11a** is a distance between the second boundary surface **31b** and the planar portion **22a**. The thickness **Lb** of the element body region **11b** is a distance between the second boundary surface **32b** and the planar portion **23a**. The thicknesses **Lb** of the element body regions **11a** and **11b** are the same.

The thicknesses **La** of the stress-relaxation spaces **31** to **33** are smaller than the thicknesses **Lb** of the element body regions **11a** and **11b**. That is, the thicknesses **Lb** of the element body regions **11a** and **11b** are larger than the thicknesses **La** of at least the stress-relaxation spaces **31** to **33**. Therefore, as compared with the thickness of the stress-

## 11

relaxation space **31**, the thickness **Lb** of the element body region **11a** is sufficiently secured between the coil conductor **21** and the coil conductor **22**. As compared with the thickness of the stress-relaxation space **32**, the thickness **Lb** of the element body region **11b** is sufficiently secured between the coil conductor **22** and the coil conductor **23**. The thicknesses **La** of the stress-relaxation spaces **31** to **33** are about 1 to 2  $\mu\text{m}$ , for example. The thicknesses **Lb** of the element body regions **11a** and **11b** are about 3 to 30  $\mu\text{m}$ , for example. A difference of the thicknesses **Lb** of the element body regions **11a** and **11b** and the thicknesses **La** of the stress-relaxation spaces **31** to **33** may be 5 to 20, for example.

Although illustration is omitted, the thickness of the element body region **11c** in the lamination direction is defined as a shortest distance of the element body region **11c** in the lamination direction, similar to the thicknesses **Lb** of the element body regions **11a** and **11b**. The thickness of the element body region **11c** in the lamination direction is the same as the thicknesses **Lb** of the element body regions **11a** and **11b**. Hereinafter, the thickness of the element body region **11c** in the lamination direction is also simply referred to as the "thickness **Lb**". The thickness **La** of the stress-relaxation space **33** is smaller than the thickness **Lb** of the element body region **11c**. That is, the thickness **Lb** of the element body region **11c** is larger than the thickness **La** of at least the stress-relaxation space **33**. Therefore, as compared with the thickness of the stress-relaxation space **33**, the thickness **Lb** of the element body region **11c** is sufficiently secured between the coil conductor **23** and the connection conductor **25**.

The stress-relaxation spaces **31** to **33** may be completely filled with the powders **31c** to **33c** and gaps may be formed between the powders **31c** to **33c**. That is, the powders **31c** to **33c** may be disposed densely in the stress-relaxation spaces **31** to **33** to be in contact with the coil conductors **21** to **23** and the element body regions **11a** to **11c** and may exist with gaps between at least one of the coil conductors **21** to **23** and the element body regions **11a** to **11c**. The gaps are formed when organic solvents contained in materials to form the stress-relaxation spaces **31** to **33** disappear at the time of firing, for example.

Even when the gaps are formed between the powders **31c** to **33c**, the thicknesses **La** of the stress-relaxation spaces **31** to **33** are defined as the distances between the first boundary surfaces **31a** to **33a** and the second boundary surfaces **31b** to **33b**, as described above. That is, the thicknesses **La** of the stress-relaxation spaces **31** to **33** are defined as the thicknesses of the stress-relaxation spaces **31** to **33** including the gaps, not the thicknesses of only the regions where the powders **31c** to **33c** other than the gaps exist.

In the element body **2**, the gaps may be formed between the element body regions **11a** to **11c** and the conductors due to a difference of shrinkage rates of the material to form the element body **2** and the material to form the conductors **21** to **25**. That is, the element body regions **11a** to **11c** may not be in contact with the conductors **21** to **25**. Even when the gaps are formed between the element body regions **11a** to **11c** and the conductors **21** to **25**, the thicknesses **Lb** of the element body regions **11a** to **11c** are defined as the shortest distances of the element body regions **11a** to **11c** in the lamination direction, as described above. When the gaps are formed between the element body regions **11a** to **11c** and the conductors **21** to **25**, the shortest distances of the element body regions **11a** to **11c** in the lamination direction are small as compared with when the gaps are not formed. For example, when the gap is not formed between the element body region **11a** and the coil conductor **22**, the thickness **Lb**

## 12

of the element body region **11a** is a distance between the second boundary surface **31b** and the planar portion **22a**. For example, when the gap is formed between the element body region **11a** and the coil conductor **22** (planar portion **22a**), the thickness **Lb** of the element body region **11a** is a distance between the second boundary surface **31b** and a boundary surface with the gap. For example, when the gap is not formed between the element body region **11b** and the coil conductor **23**, the thickness **Lb** of the element body region **11b** is a distance between the second boundary surface **32b** and the planar portion **23a**. For example, when the gap is formed between the element body region **11b** and the coil conductor **23** (planar portion **23a**), the thickness **Lb** of the element body region **11b** is a distance between the second boundary surface **32b** and a boundary surface with the gap.

Next, a course of forming conductor patterns corresponding to the individual coil conductors **21** to **23** and powder patterns corresponding to the individual stress-relaxation spaces **31** to **33** on a non-burned ceramic green sheet becoming the magnetic material layers **11** will be described.

First, the powder patterns becoming the individual stress-relaxation spaces **31** to **33** after firing are formed on the ceramic green sheet by applying paste including  $\text{ZrO}_2$ . The application of the paste is performed by screen printing, for example. The paste including  $\text{ZrO}_2$  is made by mixing  $\text{ZrO}_2$  powders and organic solvents and organic binders. Next, the conductor patterns becoming the individual coil conductors **21** to **23** after the firing are formed on the individual powder patterns formed on the ceramic green sheet by applying the conductive paste. The conductive paste is made by mixing conductor powders and organic solvents and organic binders. The application of the conductive paste is performed by the screen printing, for example. The conductor powders included in the conductor patterns become are sintered by the firing and become the coil conductors **21** to **23**. The powder patterns become the stress-relaxation spaces **31** to **33** where the powders **31c** to **33c** exist, by the firing. An average particle diameter of the powders **31c** to **33c** existing in the stress-relaxation spaces **31** to **33** is the same as an average particle diameter of the  $\text{ZrO}_2$  powders used for formation of the powder patterns before the firing.

The connection conductors **24** and **25** are formed as follows. The conductor patterns corresponding to the connection conductors **24** and **25** are formed by applying the conductive paste to the ceramic green sheet becoming the magnetic material layers **11**. The application of the conductive paste is formed by the screen printing, for example. The conductor powders included in the conductor patterns are sintered by the firing and become the connection conductors **24** and **25**. The through-hole conductors **12a** to **12d** are formed as follows. The conductive paste is filled into individual through-holes formed in the ceramic green sheet becoming the magnetic material layers **11**. The conductor powders included in the conductive paste filled into the through-holes are sintered by the firing and become the through-hole conductors **12a** to **12d**. The conductor patterns formed on the ceramic green sheet and the conductive paste filled into the through-holes are integrated. For this reason, the coil conductors **21** to **23** and the connection conductors **24** and **25** and the through-hole conductors **12a** to **12d** are formed integrally and simultaneously by the firing.

In the multilayer coil component **1** according to the first embodiment, the individual stress-relaxation spaces **31** to **33** where the powders **31c** to **33c** exist are in contact with the surfaces **21d** to **23d** of the corresponding coil conductors **21** to **23**. Therefore, the stress-relaxation spaces **31** and **32** exist between the coil conductors **21** to **23** adjacent to each other

in the lamination direction and the element body regions **11a** and **11b** located between the coil conductors **21** to **23**. The stress-relaxation spaces **31** and **32** relax the internal stress occurring in the element body **2**. The internal stress occurs due to a difference of thermal shrinkage rates of the coil conductors **21** to **23** and the element body **2**, for example. The thicknesses **La** of the stress-relaxation spaces **31** to **33** are smaller than the thicknesses **Lb** of the element body regions **11a** and **11b**. That is, the thicknesses **Lb** of the element body regions **11a** and **11b** are larger than the thicknesses **La** of at least the stress-relaxation spaces **31** and **32**. Therefore, even when the stress-relaxation spaces **31** and **32** exist between the coil conductors **21** to **23** adjacent to each other in the lamination direction and the element body regions **11a** and **11b** located between the coil conductors **21** to **23**, the element body regions **11a** and **11b** secure the sufficient thicknesses as compared with the stress-relaxation spaces **31** and **32**. As a result, the thicknesses **Lb** of the element body regions **11a** and **11b** are sufficiently secured, and the internal stress occurring in the element body **2** is relaxed.

In the multilayer coil component **1**, the stress-relaxation spaces **31** to **33** are in contact with the surfaces **21d** to **23d** of the coil conductors **21** to **23**. That is, the individual stress-relaxation spaces **31** to **33** are formed on the surfaces **21d** to **23d** of the corresponding coil conductors **21** to **23**. When the stress-relaxation spaces **31** to **33** are formed on the surfaces **21d** to **23d**, the individual stress-relaxation spaces **31** to **33** are formed easily and the thicknesses of the element body regions **11a** and **11b** are secured more easily, as compared with when the stress-relaxation spaces **31** to **33** are formed on both the surfaces **21d** to **23d** and the surfaces **21e**, **23e**. The surfaces **21e** to **23e** on which the stress-relaxation spaces **31** to **33** are not formed are coupled to the element body **2** not via the stress-relaxation spaces **31** to **33**. Therefore, coupling strength of the surfaces **21e** to **23e** and the element body **2** is high.

In the multilayer coil component **1**, the stress-relaxation spaces **31** to **33** are in contact with the planar surfaces **21d** to **23d**. That is, because the surfaces **21d** to **23d** on which the stress-relaxation spaces **31** to **33** are formed have planar shapes, the stress-relaxation spaces **31** to **33** are formed easily.

In the multilayer coil component **1**, the average particle diameter of the powders **31c** to **33c** is  $0.1 \mu\text{m}$  or less. In which case, because fluidity of the powders **31c** to **33c** is superior, the powders **31c** to **33c** flexibly follow the behavior according to the difference of the thermal shrinkage rates of the element body **2** and the coil conductors **21** to **23**. As a result, the internal stress occurring in the element body **2** is relaxed more surely.

In the multilayer coil component **1**, the materials of the powders **31c** to **33c** are  $\text{ZrO}_2$ .  $\text{ZrO}_2$  is hard to affect the ferrite material included in the element body **2**. Because the melting point of  $\text{ZrO}_2$  is higher than a firing temperature of the ferrite material included in the element body **2**,  $\text{ZrO}_2$  exists surely as the powders.

In the multilayer coil component **1**, the individual coil conductors **21** to **23** contain the metal oxide. When the coil conductors **21** to **23** contain the metal oxide, the shrinkage rate at the time of firing the conductive paste configuring the coil conductors **21** to **23** is small as compared with when the coil conductors **21** to **23** do not contain the metal oxide. For this reason, the cross-sections of the coil conductors **21** to **23** are large. Therefore, even when the cross-sections of the coil

conductors **21** to **23** are large, the stress-relaxation spaces **31** to **33** relax the internal stress occurring in the element body **2**.

In the multilayer coil component **1**, because the stress-relaxation space is not formed in each of the connection conductors **24** and **25**, adhesion of the connection conductors **24** and **25** and the magnetic material layers **11** is superior. Therefore, intrusion of a plating solution from the ends **24a** and **25a** of the connection conductors **24** and **25**, that is, the portions of the connection conductors **24** and **25** exposed to the end surfaces **2a** and **2b** is suppressed.

## Second Embodiment

A multilayer coil component **1A** according to a second embodiment will be described with reference to FIGS. **8** to **10**. FIG. **8** is an exploded perspective view of the multilayer coil component according to the second embodiment. FIGS. **9A** and **9B** are plan views illustrating connection conductors. FIG. **10** is a cross-sectional view of the multilayer coil component according to the second embodiment. FIGS. **9A** and **9B** correspond to FIG. **6**. In FIG. **8**, illustration of a plurality of magnetic material layers and external electrodes is omitted. In FIG. **10**, illustration of the external electrodes is omitted. Because a perspective view of the multilayer coil component **1A** according to the second embodiment is the same as that of FIG. **1**, illustration is omitted.

As illustrated in FIGS. **8** to **10**, the multilayer coil component **1A** includes an element body **2**, a pair of external electrodes **4** and **5** (refer to FIG. **1**), a plurality of coil conductors **21** to **23**, a plurality of connection conductors **24** and **25**, and a plurality of stress-relaxation spaces **31** to **33**, similar to the multilayer coil component **1**. The multilayer coil component **1A** is different from the multilayer coil component **1** in that the multilayer coil component **1A** includes stress-relaxation spaces **34** and **35** are in contact with the connection conductors **24** and **25**. The stress-relaxation spaces **34** and **35** are spaces where powders **34c** and **35c** exist, respectively (refer to FIG. **8**). The stress-relaxation spaces **34** and **35** exist between the corresponding connection conductors **24** and **25** and element body regions in the element body **2** and relax internal stress occurring in the element body **2**. Materials of the powders **34c** and **35c** are  $\text{ZrO}_2$ , for example. An average particle diameter of the powders **34c** and **35c** is  $0.1 \mu\text{m}$  or less, for example.

As illustrated in FIG. **8**, the stress-relaxation space **34** is located between the connection conductor **24** and the coil conductor **21** in a lamination direction. As illustrated in FIG. **9A**, the stress-relaxation space **34** is formed on a surface **24d** of the connection conductor **24** (refer to FIG. **10**). The surface **24d** is a lower surface of the connection conductor **24** in the lamination direction. That is, the surface **24d** is a surface close to a side surface **2d** in the lamination direction. The stress-relaxation space **34** is formed along a portion other than an end **T5** and an end **24a** of the connection conductor **24**. That is, the stress-relaxation space **34** does not cover the end **T5** and the end **24a** of the connection conductor **24**. The end **T5** is a connection portion with a through-hole conductor **12a**. The end **24a** is a connection portion with the external electrode **4**. The stress-relaxation space **34** is formed not to protrude from the connection conductor **24**, when viewed from the lamination direction.

The stress-relaxation space **35** is located between the connection conductor **25** and the coil conductor **23** in the lamination direction. As illustrated in FIG. **9B**, the stress-relaxation space **35** is formed on a surface **25d** of the connection conductor **25** (refer to FIG. **10**). The surface **25d**

is a lower surface of the connection conductor 25 in the lamination direction. That is, the surface 25d is a surface close to the side surface 2d in the lamination direction. The stress-relaxation space 35 is formed along a portion other than an end T6 and an end 25a of the connection conductor 25. That is, the stress-relaxation space 35 does not cover the end T6 and the end 25a of the connection conductor 25. The end T6 is a connection portion with a through-hole conductor 12d. The end 25a is a connection portion with the external electrode 4. The stress-relaxation space 35 is formed not to protrude from the connection conductor 25, when viewed from the lamination direction.

As illustrated in FIG. 10, the stress-relaxation space 34 includes a first boundary surface 34a with the connection conductor 24 and a second boundary surface 34b with an element body region 11d. The first boundary surface 34a is in contact with the surface 24d of the connection conductor 24. The second boundary surface 34b is in contact with the element body region 11d. In the second embodiment, the element body region 11d is interposed by the coil conductor 21 and the stress-relaxation space 34. In the first embodiment, the element body region 11d is interposed by the coil conductor 21 and the connection conductor 24. The first boundary surface 34a and the second boundary surface 34b oppose each other in the lamination direction.

The stress-relaxation space 35 includes a first boundary surface 35a with the connection conductor 25 and a second boundary surface 35b with an element body region 11e. The element body region 11e is located between the connection conductor 25 and the side surface 2d. The first boundary surface 35a is in contact with a surface 25d of the connection conductor 25. The second boundary surface 35b is in contact with the element body region 11e. The first boundary surface 35a and the second boundary surface 35b oppose each other in the lamination direction.

Although illustration is omitted, the thicknesses of the stress-relaxation spaces 34 and 35 in the lamination direction are defined as distances between the first boundary surfaces 34a and 35a and the second boundary surfaces 34b and 35b opposing each other, similar to the thicknesses La of the stress-relaxation spaces 34 and 35. Hereinafter, the thicknesses of the stress-relaxation spaces 34 and 35 in the lamination direction are also referred to as the “thicknesses La”. The thickness La of the stress-relaxation space 34 is a distance between the first boundary surface 34a and the second boundary surface 34b. The thickness La of the stress-relaxation space 35 is a distance between the first boundary surface 35a and the second boundary surface 35b. The thicknesses La of the stress-relaxation spaces 34 and 35 are the same as the thicknesses La of the stress-relaxation spaces 31 to 33.

Although illustration is omitted, the thickness of the element body region 11d in the lamination direction is defined as a shortest distance of the element body region 11d in the lamination direction, similar to the thicknesses Lb of the element body regions 11a to 11c. The thickness of the element body region 11d in the lamination direction is the same as the thicknesses Lb of the element body regions 11a to 11c. Hereinafter, the thickness of the element body region 11d in the lamination direction is also referred to as the “thickness Lb”. The thickness La of the stress-relaxation space 34 is smaller than the thickness Lb of the element body region 11d. That is, the thickness Lb of the element body region 11d is larger than the thickness La of at least the stress-relaxation space 34. Therefore, as compared with the thickness of the stress-relaxation space 34, the thickness Lb

of the element body region 11d is sufficiently secured between the coil conductor 21 and the connection conductor 24.

The stress-relaxation spaces 34 and 35 may be completely filled with the powders 34c and 35c and gaps may be formed between the powders 34c and 35c. Even when the gaps are formed between the powders 34c and 35c, the thicknesses La of the stress-relaxation spaces 34 and 35 are defined as described above. That is, the thicknesses La of the stress-relaxation spaces 34 and 35 are defined as the thicknesses of the stress-relaxation spaces 34 and 35 including the gaps, not the thicknesses of only the regions where the powders 34c and 35c other than the gaps exist.

Similar to the first embodiment, in the second embodiment, the thicknesses Lb of the element body regions 11a and 11b are sufficiently secured, and the internal stress occurring in the element body 2 is relaxed.

In the second embodiment, because the individual stress-relaxation spaces 34 and 35 are formed in the corresponding connection conductors 24 and 25, the internal stress occurring in the element body 2 is further relaxed. The thickness Lb of the element body region 11d is larger than the thickness of at least the stress-relaxation space 34. Therefore, even when the stress-relaxation space 34 exists between the connection conductor 24 and the coil conductor 21 adjacent to each other in the lamination direction, the element body region 11d secures the sufficient thickness as compared with the stress-relaxation space 34.

In the second embodiment, the stress-relaxation spaces 34 and 35 are formed not to cover the ends 24a and 25a of the connection conductors 24 and 25, that is, portions of the connection conductors 24 and 25 exposed to end surfaces 2a and 2b. Because the ends 24a and 25a and the element body 2 are coupled not via the stress-relaxation spaces 34 and 35, adhesion of the ends 24a and 25a and the element body 2 is superior. Therefore, intrusion of a plating solution from the ends 24a and 25a is suppressed.

### Third Embodiment

A multilayer coil component 1B according to a third embodiment will be described with reference to FIGS. 11 to 16. FIG. 11 is an exploded perspective view of the multilayer coil component according to the third embodiment. FIGS. 12 to 14 are plan views illustrating coil conductors. FIG. 15 is a cross-sectional view of the multilayer coil component according to the third embodiment. FIG. 15 corresponds to FIG. 6. FIG. 16 is a diagram illustrating a part of FIG. 15. In FIG. 11, illustration of a plurality of magnetic material layers and external electrodes is omitted. In FIG. 15, illustration of the external electrodes is omitted. Because a perspective view of the multilayer coil component 1B according to the third embodiment is the same as that of FIG. 1, illustration is omitted.

As illustrated in FIGS. 11 to 16, the multilayer coil component 1B includes an element body 2, a pair of external electrodes 4 and 5 (refer to FIG. 1), a plurality of coil conductors 21 to 23, and a plurality of connection conductors 24 and 25, similar to the multilayer coil component 1. The multilayer coil component 1B is different from the multilayer coil component 1 in that the multilayer coil component 1B includes a plurality of stress-relaxation spaces 41 to 43, instead of the plurality of stress-relaxation spaces 31 to 33.

The individual stress-relaxation spaces 41 to 43 are in contact with the corresponding coil conductors 21 to 23. The stress-relaxation spaces 41 to 43 are spaces where powders

41c, 42c, and 43c exist, respectively. The individual stress-relaxation spaces 41 to 43 exist between the corresponding coil conductors 21 to 23 and element body regions in the element body 2 and relax internal stress occurring in the element body 2. Materials of the powders 41c, 42c, and 43c are ZrO<sub>2</sub>, for example. An average particle diameter of the powders 41c, 42c, and 43c is 0.1 μm or less, for example.

As illustrated in FIG. 11, the stress-relaxation space 41 is located between the connection conductor 24 and the coil conductor 21 in a lamination direction. As illustrated in FIG. 12, the stress-relaxation space 41 is formed on a surface 21e of the coil conductor 21 (refer to FIG. 16). The surface 21e is an upper surface of the coil conductor 21 in the lamination direction. That is, the surface 21e is a surface close to a side surface 2c in the lamination direction. The stress-relaxation space 41 is formed along a portion other than an end E1 of the coil conductor 21. That is, the stress-relaxation space 41 does not cover the end E1 of the coil conductor 21. The end E1 is a connection portion with a through-hole conductor 12a. The stress-relaxation space 41 is formed not to protrude from the coil conductor 21, when viewed from the lamination direction.

The stress-relaxation space 42 is located between the coil conductor 21 and the coil conductor 22 in the lamination direction. As illustrated in FIG. 13, the stress-relaxation space 42 is formed on a surface 22e of the coil conductor 22 (refer to FIG. 16). The surface 22e is an upper surface of the coil conductor 21 in the lamination direction. That is, the surface 22e is a surface close to the side surface 2c. The stress-relaxation space 42 is formed along a portion other than an end T2 of the coil conductor 22. That is, the stress-relaxation space 42 does not cover the end T2 of the coil conductor 22. The end T2 is a connection portion with a through-hole conductor 12b. The stress-relaxation space 42 is formed not to protrude from the coil conductor 22, when viewed from the lamination direction.

The stress-relaxation space 43 is located between the coil conductor 22 and the coil conductor 23 in the lamination direction. As illustrated in FIG. 14, the stress-relaxation space 43 is formed on a surface 23e of the coil conductor 23 (refer to FIG. 16). The surface 23e is an upper surface of the coil conductor 21 in the lamination direction. That is, the surface 23e is a surface close to the side surface 2c. The stress-relaxation space 43 is formed along a portion other than an end T4 of the coil conductor 23. That is, the stress-relaxation space 43 does not cover the end T4 of the coil conductor 23. The end T4 is a connection portion with a through-hole conductor 12c. The stress-relaxation space 43 is formed not to protrude from the coil conductor 23, when viewed from the lamination direction.

As illustrated in FIG. 15, in the third embodiment, an element body region 11a is interposed by the coil conductor 21 and the stress-relaxation space 42. An element body region 11b is interposed by the coil conductor 22 and the stress-relaxation space 43. An element body region 11c is interposed by the coil conductor 23 and the connection conductor 25. An element body region 11d is interposed by the connection conductor 24 and the stress-relaxation space 41.

Referring to FIG. 16, cross-sectional configurations of each of the coil conductors 21 to 23 and each of the stress-relaxation spaces 41 to 43 will be described. In FIG. 16, regions including parts (portions close to an end surface 2b of the element body 2) of the coil conductors 21 to 23 in FIG. 15 are expanded. Because configurations of regions including portions of the coil conductors 21 to 23 close to an end surface 2a of the element body 2 in FIG. 15 are the same

as the configurations illustrated in FIG. 16, illustration is omitted. In the third embodiment, a direction toward the side surface 2c from a side surface 2d is one direction D3 of the lamination direction and a direction toward the side surface 2d from the side surface 2c is the other direction D4 of the lamination direction. That is, in the third embodiment, the surfaces 21e, 22e, and 23e are first surfaces facing one direction D3 of the lamination direction and surfaces 21d, 22d, and 23d are second surfaces facing the other direction D4 of the lamination direction.

As illustrated in FIG. 16, the stress-relaxation space 41 includes a first boundary surface 41b with the coil conductor 21 and a second boundary surface 41a with the element body region 11d. The first boundary surface 41b is in contact with the surface 21e of the coil conductor 21. That is, the first boundary surface 41b is in contact with a planar portion 21a and inclined portions 21b and 21c. In the third embodiment, the first boundary surface 41b continuously is in contact with the planar portion 21a and the inclined portions 21b and 21c. The stress-relaxation space 41 covers the planar portion 21a and the inclined portions 21b and 21c integrally. The second boundary surface 41a is in contact with the element body region 11d. The first boundary surface 41b and the second boundary surface 41a oppose each other in the lamination direction.

The stress-relaxation space 42 includes a first boundary surface 42b with the coil conductor 22 and a second boundary surface 42a with an element body region 11a. The first boundary surface 42b is in contact with the surface 22e of the coil conductor 22. That is, the first boundary surface 42b is in contact with a planar portion 22a and inclined portions 22b and 22c. In the third embodiment, the first boundary surface 42b continuously is in contact with the planar portion 22a and the inclined portions 22b and 22c. The stress-relaxation space 42 covers the planar portion 22a and the inclined portions 22b and 22c integrally. The second boundary surface 42a is in contact with the element body region 11a. The first boundary surface 42b and the second boundary surface 42a oppose each other in the lamination direction.

The stress-relaxation space 43 includes a first boundary surface 43b with the coil conductor 23 and a second boundary surface 43a with the element body region 11b. The first boundary surface 43b is in contact with the surface 23e of the coil conductor 23. That is, the first boundary surface 43b is in contact with a planar portion 23a and inclined portions 23b and 23c. In the third embodiment, the first boundary surface 43b continuously is in contact with the planar portion 23a and the inclined portions 23b and 23c. The stress-relaxation space 43 covers the planar portion 23a and the inclined portions 23b and 23c integrally. The second boundary surface 43a is in contact with the element body region 11b. The first boundary surface 43b and the second boundary surface 43a oppose each other in the lamination direction.

The thicknesses (hereinafter, simply referred to as the “thicknesses Lc”) of the individual stress-relaxation spaces 41 to 43 in the lamination direction are defined as distances between the first boundary surfaces 41b to 43b and the second boundary surfaces 41a to 43a opposing each other. In the third embodiment, the thickness Lc of the stress-relaxation space 41 is a distance between the first boundary surface 41b and the second boundary surface 41a. The thickness Lc of the stress-relaxation space 42 is a distance between the first boundary surface 42b and the second boundary surface 42a. The thickness Lc of the stress-relaxation space 43 is a distance between the first boundary

surface **43b** and the second boundary surface **43a**. The thicknesses **Lc** of the individual stress-relaxation spaces **41** to **43** are the same.

The thicknesses (hereinafter, simply referred to as the "thicknesses **Ld**") of the individual element body regions **11a** and **11b** in the lamination direction are defined as shortest distances of the element body regions **11a** and **11b** in the lamination direction. In the third embodiment, the thickness **Ld** of the element body region **11a** is a distance between the second boundary surface **42a** and the surface **21d**. The thickness **Ld** of the element body region **11b** is a distance between the second boundary surface **43a** and the surface **22d**. The thicknesses **Ld** of the individual element body regions **11a** and **11b** are the same.

The thicknesses **Lc** of the individual stress-relaxation spaces **41** to **43** are smaller than the thicknesses **Ld** of the individual element body regions **11a** and **11b**. That is, the thicknesses **Ld** of the element body regions **11a** and **11b** are larger than the thicknesses **Lc** of at least the stress-relaxation spaces **41** to **43**. Therefore, as compared with the thickness of the stress-relaxation space **41**, the thickness **Ld** of the element body region **11a** is sufficiently secured between the coil conductor **21** and the coil conductor **22**. As compared with the thickness of the stress-relaxation space **42**, the thickness **Ld** of the element body region **11b** is sufficiently secured between the coil conductor **22** and the coil conductor **23**. The thicknesses **L** of the stress-relaxation spaces **41** to **43** are about 1 to 2  $\mu\text{m}$ , for example. Meanwhile, the thicknesses **Ld** of the element body regions **11a** and **11b** are about 3 to 30  $\mu\text{m}$ , for example. A difference of the thicknesses **Lc** of the element body regions **11a** and **11b** and the thicknesses **Ld** of the stress-relaxation spaces **41** to **43** may be 5 to 20, for example.

Although illustration is omitted, the thickness of the element body region **11d** in the lamination direction is defined as a shortest distance of the element body region **11d** in the lamination direction, similar to the thicknesses **Lc** of the element body regions **11a** and **11b**. The thickness of the element body region **11d** in the lamination direction is the same as the thicknesses **Lc** of the element body regions **11a** and **11b**. Hereinafter, the thickness of the element body region **11d** in the lamination direction is also simply referred to as the "thickness **Lc**". The thickness **La** of the stress-relaxation space **41** is smaller than the thickness **Ld** of the element body region **11d**. That is, the thickness **Ld** of the element body region **11d** is larger than the thickness **Lc** of at least the stress-relaxation space **41**. Therefore, as compared with the thickness of the stress-relaxation space **41**, the thickness **Ld** of the element body region **11d** is sufficiently secured between the coil conductor **21** and the connection conductor **24**.

The stress-relaxation spaces **41** to **43** may be completely filled with the powders **41c** to **43c** and gaps may be formed between the powders **41c** to **43c**, similar to the first and second embodiments. Even when the gaps are formed between the powders **41c** to **43c**, the thicknesses **Lc** of the stress-relaxation spaces **41** to **43** are defined as described above. That is, the thicknesses **Lc** of the stress-relaxation spaces **41** to **43** are defined as the thicknesses of the stress-relaxation spaces **41** to **43** including the gaps, not the thicknesses of only the regions where the powders **41c** to **43c** other than the gaps exist.

The element body regions **11a**, **11b**, and **11d** may not be in contact with the conductors **21** to **25**, similar to the element body regions **11a** to **11c**. Even when the gaps are formed between the element body regions **11a** to **11c** and the conductors **21** to **25**, the thicknesses **Ld** of the element body

regions **11a**, **11b**, and **11d** are defined as the shortest distances of the element body regions **11a**, **11b**, and **11d** in the lamination direction, as described above. When the gaps are formed between the element body regions **11a** to **11c** and the conductors **21** to **25**, the shortest distances of the element body regions **11a**, **11b**, and **11d** in the lamination direction become small as compared with when the gaps are not formed. For example, when the gap is not formed between the element body region **11a** and the coil conductor **21**, the thickness **Ld** of the element body region **11a** is a distance between the second boundary surface **42a** and the surface **21d**. For example, when the gap is formed between the element body region **11a** and the coil conductor **21** (surface **21d**), the thickness **Ld** of the element body region **11a** is a distance between the second boundary surface **42a** and a boundary surface with the gap. For example, when the gap is not formed between the element body region **11b** and the coil conductor **22**, the thickness **Ld** of the element body region **11b** is a distance between the second boundary surface **43a** and the surface **22d**. For example, when the gap is formed between the element body region **11b** and the coil conductor **22** (surface **22d**), the thickness **Ld** of the element body region **11b** is a distance between the second boundary surface **43a** and a boundary surface with the gap.

Next, a course of forming conductor patterns corresponding to the individual coil conductors **21** to **23** and powder patterns corresponding to the individual stress-relaxation spaces **41** to **43** on a non-burned ceramic green sheet becoming magnetic material layers **11** will be described. Because a method of forming the individual connection conductors **24** and **25** and a method of forming the individual through-hole conductors **12a** to **12d** are the same as those in the first embodiment, explanation thereof is omitted.

First, the conductor patterns becoming the individual coil conductors **21** to **23** after firing are formed on the ceramic green sheet by applying the conductive paste. The application of the conductive paste is performed by screen printing, for example. The conductive paste is made by mixing conductor powders and organic solvents and organic binders. Next, the powder patterns becoming the individual stress-relaxation spaces **41** to **43** after the firing are formed on the individual conductor patterns formed on the ceramic green sheet by applying paste including  $\text{ZrO}_2$ . The application of the paste is performed by the screen printing, for example. The paste including  $\text{ZrO}_2$  is made by mixing  $\text{ZrO}_2$  powders and organic solvents and organic binders. The conductor powders included in the conductor patterns become are sintered by the firing and become the coil conductors **21** to **23**. The powder patterns become the stress-relaxation spaces **41** to **43** where the powders **41c** to **43c** exist, by the firing. An average particle diameter of the powders **41c** to **43c** existing in the stress-relaxation spaces **41** to **43** is the same as an average particle diameter of the  $\text{ZrO}_2$  powders used for formation of the powder patterns before the firing.

In the multilayer coil component **1B** according to the third embodiment, the individual stress-relaxation spaces **41** to **43** where the powders **41c** to **43c** exist are in contact with the surfaces **21e** to **23e** of the corresponding coil conductors **21** to **23**. Therefore, the stress-relaxation spaces **42** and **43** exist between the coil conductors **21** to **23** adjacent to each other in the lamination direction and the element body regions **11a** and **11b** located between the coil conductors **21** to **23**. The stress-relaxation spaces **41** to **43** relax the internal stress occurring in the element body **2**. The internal stress occurs due to a difference of thermal shrinkage rates of the coil conductors **21** to **23** and the element body **2**, for example.

## 21

The thicknesses  $L_c$  of the stress-relaxation spaces **41** to **43** are smaller than the thicknesses  $L_d$  of the element body regions **11a** and **11b**. That is, the thicknesses  $L_d$  of the element body regions **11a** and **11b** are larger than the thicknesses  $L_e$  of at least the stress-relaxation spaces **41** to **43**. Therefore, even when the stress-relaxation spaces **42** and **43** exist between the coil conductors **21** to **23** adjacent to each other in the lamination direction and the element body regions **11a** and **11b** located between the coil conductors **21** to **23**, the element body regions **11a** and **11b** secure the sufficient thicknesses as compared with the stress-relaxation spaces **42** and **43**. As a result, the thicknesses  $L_d$  of the element body regions **11a** and **11b** are sufficiently secured, and the internal stress occurring in the element body **2** is relaxed.

In the multilayer coil component **1B**, the stress-relaxation spaces **41** to **43** are in contact with the planar portions **21a** to **23a** and the inclined portions **21b** to **23b** and **21c** to **23c**. For this reason, the internal stress occurring in the element body **2** is relaxed surely.

The various embodiments have been described. However, the present invention is not limited to the embodiments and various changes, modifications, and applications can be made without departing from the gist of the present invention.

In the embodiments, the stress-relaxation spaces **31** to **33** and **41** to **43** are in contact with the surfaces facing one direction  $D_1$  and  $D_3$  of the lamination direction in the corresponding coil conductors **21** to **23**. However, the present invention is not limited thereto. For example, the stress-relaxation spaces may be in contact with the surfaces facing one direction  $D_1$  and  $D_3$  of the lamination direction and the surfaces facing the other directions  $D_2$  and  $D_4$  of the lamination direction in the coil conductors **21** to **23**. The stress-relaxation spaces **31** to **33** and **41** to **43** may be in contact with the parts of the surfaces of the corresponding coil conductors **21** to **23** and may be in contact with the entire portions of the surfaces of the corresponding coil conductors **21** to **23**. The stress-relaxation spaces **31** to **33** and **41** to **43** may be formed to surround the surfaces of the corresponding coil conductors **21** to **23**. In the embodiments, the stress-relaxation spaces **31** to **33** and **41** to **43** are formed not to protrude from the corresponding coil conductors **21** to **23**, when viewed from the lamination direction. However, the present invention is not limited thereto. For example, the stress-relaxation spaces **31** to **33** and **41** to **43** may be formed to protrude from the corresponding coil conductors **21** to **23**, when viewed from the lamination direction. In the embodiments, the stress-relaxation spaces **34** and **35** are formed not to protrude from the connection conductors **24** and **25**, when viewed from the lamination direction. However, the present invention is not limited thereto. For example, the stress-relaxation spaces **34** and **35** may be formed to protrude from the connection conductors **24** and **25**, when viewed from the lamination direction.

In the embodiments, the cross-sectional shapes of the coil conductors **21** to **23** are approximately the trapezoidal shapes. However, the present invention is not limited thereto. For example, the cross-sectional shapes of the coil conductors **21** to **23** may be approximately rectangular shapes.

In the embodiments, the thicknesses of the coil conductors **21** to **23** and the connection conductors **24** and **25** in the lamination direction are approximately the same. However, the present invention is not limited thereto. For example, the thicknesses of the connection conductors **24** and **25** in the lamination direction may be smaller than the thicknesses of

## 22

the coil conductors **21** to **23**. In this case, the stress is suppressed from occurring in the element body **2** due to the connection conductors **24** and **25**. When the thickness of the connection conductor **24** in the lamination direction is small, electrical resistance of the connection conductor **24** increases. For this reason, the electrical resistance of the connection conductor **24** may be decreased by placing the plurality of connection conductors **24** side by side in the lamination direction. Likewise, the electrical resistance of the connection conductor **25** may be decreased by placing the plurality of connection conductors **25** side by side in the lamination direction.

In the embodiments, the materials of the powders **31c** to **35c** and **41c** to **43c** are  $ZrO_2$ , for example. However, the present invention is not limited thereto. For example, the materials of the powders **31c** to **35c** and **41c** to **43c** may be ferrite materials having a higher firing temperature than the ferrite material configuring the element body **2**. In which case, the stress-relaxation spaces **31** to **35** and **41** to **43** where the powders **31c** to **35c** and **41c** to **43c** exist also function as magnetic materials. The materials of the powders configuring the stress-relaxation spaces **31** to **33** and **41** to **43** may be materials having higher permittivity than the element body **2**. In which case, stray capacitance occurring between the coil conductors **21** to **23** is reduced.

In the third embodiment, the stress-relaxation spaces may be formed in the connection conductors **24** and **25**.

What is claimed is:

1. A multilayer coil component comprising:  
an element body that includes a magnetic material;  
a coil configured to include a plurality of internal conductors separated from each other in a first direction in the element body and electrically connected to each other; and  
a plurality of stress-relaxation spaces configured to be in contact with surfaces of the plurality of internal conductors,

wherein  
the element body includes element body regions located between each pair of one of the plurality of internal conductors and one of the plurality of stress-relaxation spaces adjacent to each other in the first direction, each of the plurality of stress-relaxation spaces includes non-sintered powders in a final state of the each of the plurality of stress-relaxation spaces, a first boundary surface with an internal conductor of the plurality of internal conductors, and a second boundary surface with one of the element body regions,

the first boundary surface and the second boundary surface oppose each other in the first direction, a distance between the first boundary surface and the second boundary surface is smaller than a thickness of each of the element body regions in the first direction.

2. The multilayer coil component according to claim 1, wherein each of the plurality of internal conductors includes a first surface facing one direction of the first direction and a second surface facing the other direction of the first direction, and

the first surface is in contact with the first boundary surface.

3. The multilayer coil component according to claim 2, wherein the first surface has a planar shape.

4. The multilayer coil component according to claim 2, wherein the first surface includes a first surface portion extending in a direction orthogonal to the first direction and a second surface portion inclined with respect to the first direction and the first surface portion, and

the each stress-relaxation space is in contact with the first surface portion and the second surface portion.

**5. The multilayer coil component according to claim 2, wherein the second surface does not contact the plurality of stress-relaxation spaces.**

5

**6. The multilayer coil component according to claim 1, wherein an average particle diameter of the powders is 0.1  $\mu\text{m}$  or less.**

**7. The multilayer coil component according to claim 1, wherein materials of the powders are  $\text{ZrO}_2$ .**

10

**8. The multilayer coil component according to claim 1, wherein each of the plurality of internal conductors contains metal oxide.**

\* \* \* \* \*